

1

3,723,118

### DIFFUSION TRANSFER PROCESS FOR PHOTOGRAPHIC SILVER HALIDE EMULSION

Haruhiko Iwano, Mitsugu Tanaka, Tetsuo Otsuki, and Atsushi Arai, Kanagawa, Japan, assignors to Fuji Photo Film Co., Ltd., Kanagawa, Japan

No Drawing. Filed June 8, 1971, Ser. No. 150,932  
Claims priority, application Japan, June 8, 1970,  
45/49,338

U.S. Cl. 96—29

Int. Cl. G03c 5/54

12 Claims

#### ABSTRACT OF THE DISCLOSURE

A high speed diffusion transfer process which comprises processing an exposed photographic silver halide material with a processing solution containing a compound represented by the following general formula or acid salt thereof:



wherein X is a lower alkenyl or a lower alkenoxy group, R<sub>1</sub> is hydrogen, or a lower alkyl group, and R<sub>2</sub>, R<sub>3</sub> and R<sub>4</sub> each is hydrogen, a lower alkyl group, a lower alkenyl group or a lower alkoxy group, in which the term "lower" indicates that the total number of carbon atoms contained is not more than 4.

#### FIELD OF THE INVENTION

The present invention relates to a process for processing an exposed photographic silver halide light-sensitive material. More particularly, the present invention relates to a process for processing exposed silver halide photographic material by diffusion transfer process.

In diffusion transfer process, a latent image formed in a negative emulsion layer by imagewise exposure is developed and, simultaneously, a residual unexposed silver halide, i.e., undeveloped silver halide, in the negative emulsion layer, is reacted with a silver halide solvent to form a soluble silver complex in an amount corresponding to the amount of the exposure. Such soluble, silver complex is reduced in a print-receiving layer which is brought into contact with the exposed silver halide emulsion layer and contains a suitable silver precipitating layer, whereby the reduced silver is precipitated to give the desired positive image.

#### OBJECT OF THE INVENTION

An object of the present invention is to prepare a processing solution for a high speed diffusion transfer process, which is suitable for forming satisfactory images from a silver halide emulsion exposed to a small quantity of light, for example, of exposure index ASA 1,000.

The processing solution to be employed in the diffusion transfer process according to the present invention is a viscous liquid which is uniformly spread between the negative and positive layers, and develops a latent image in the silver halide emulsion layer, even when formed by a small quantity of exposure index more than ASA 1,000, followed by the same step as above to form positive images. Moreover, it is desirable to finish the processings to form the positive image within short periods of time, that is, within 1 minute.

Therefore, in the high speed diffusion transfer process as described above, it is necessary to use a highly active developing agent to develop rapidly a weak latent image formed by little exposure. Furthermore, as the solvent for silver halide to form a soluble silver complex there

2

are thiosulfates, thiocyanates and the like. In addition, there may be added into the processing solution alkaline agents, normally employed additives, such as potassium bromide, and antifoggants such as 6-nitro-benzimidazole, as well as a viscosity-increasing agent, such as carboxymethyl cellulose, hydroxyethyl cellulose and the like.

An object of the present invention is to prepare a processing solution for use in a high speed diffusion transfer process which is suitable for the purpose of forming a satisfactory positive image from a silver halide emulsion which has been exposed to small quantities of light, for example, to light showing an exposure index of ASA 1,000.

More particularly, this invention provides highly active developing agents suitable for use in processing solutions employed in the above-described high speed diffusion transfer process.

#### DESCRIPTION OF THE PREFERRED EMBODIMENT

Thus, it has now been found that the above objects can be attained by a developing agent represented by the following formula:



wherein X is a lower alkenyl or a lower alkenoxy group, R<sub>1</sub> is hydrogen or a lower alkyl group, and R<sub>2</sub>, R<sub>3</sub> and R<sub>4</sub> each is hydrogen, a lower alkyl group, a lower alkenyl group, or a lower alkoxy group, the term "lower" indicating that the total number of carbon atoms is not more than 4.

The compounds of the above-described formula to be employed according to the present invention may be used in either the form of a free amine, as shown by the general formula itself, or in the more stable form of acid addition salts, such as sulfates and hydrochlorides.

Although many analogous p-aminophenols such as Metol (i.e., N-methyl-p-aminophenol sulfate) have been known and practically employed, the compounds of the above-described general formula are characterized by having a substituent X, and it has now been found that the combination of these compounds with the high diffusion transfer process can afford particularly preferred results.

As described above, the images obtained by the high speed diffusion transfer process using, as a developing agent, a compound of the above-described general formula can yield a satisfactory positive image. Also, the compounds represented by the general formula are very soluble in water. Since a quantity of the highly active developing agent is to be employed in the processing solution of the high speed diffusion transfer process, the great solubility in water can be extremely advantageous.

Furthermore, the compounds of the general formula may be used singly as highly active developing agents or may be used together with other reducing agents, such as phenols, such as cresol, and hydroxylamines, such as N,N-diethylhydroxylamine.

In both cases, there may be obtained a good positive image by the diffusion transfer process.

As practical examples of the silver halide developing agents of the invention, there are the following:

- (1) 4-amino-2-allylphenol,
- (2) 4-amino-2-allyloxyphenol,
- (3) 4-amino-2,6-diallylphenol,
- (4) 4-amino-2-allyl-3,5-dimethylphenol, and
- (5) 4-methylamino-2-allylphenol.

Typical methods for preparing the compounds of the above-described general formula are shown as follows:

Synthesis 1 (4-amino-2-allylphenol hydrochloride)

While a solution consisting of 97 g. of sulfanilic acid, 39.2 g. of sodium carbonate monohydrate and 1 liter of water was maintained at 8° C., 168 ml. of concentrated hydrochloric acid and then 40.6 g. of sodium nitrite dissolved in a small amount of water were added to obtain a reaction mixture containing white diazonium salt.

The resulting mixture was added to a solution composed of 112 g. of caustic soda, 164 g. of sodium carbonate monohydrate, 75 g. of 2-allylphenol and 2 liters of water with stirring, wherein the temperature of the reaction mixture should be kept below 5° C. in a water bath. After the addition, the water bath was removed and, after stirring for an hour, 400 g. of sodium hydro-sulfite was added thereto followed by heating to 70° C. to provide precipitated white crystals of the amine. After cooling, the crystalline amine was collected and converted into its hydrochloride, whereby 67 g. of 4-amino-2-allylphenol hydrochloride, as colorless crystals having a melting point of from 177 to 190° C. (decomposed), was obtained in a yield of 64.4%.

Synthesis 2 (4-amino-2,6-diallylphenol hydrochloride)

In a manner similar to Synthesis 1, 2,6-diallylphenol was coupled with a diazonium salt of sulfanilic acid followed by treatment with sodium hydrosulfite. The resulting amine was converted into its hydrochloride to obtain the desired product, as colorless needles having a melting point of from 125 to 165° C. (decomposed), in a yield of 51.0%.

Synthesis 3 (4-amino-2-allyl-3,5-dimethylphenol hydrochloride)

In a manner similar to Synthesis 1, 2-allyl-3,5-dimethylphenol was coupled with a diazonium salt of sulfanilic acid followed by treatment with sodium hydrosulfite. The resulting amine was formed into its hydrochloride to obtain the desired product as colorless crystals having a melting point of from 236 to 237° C. in a yield of 55.1%.

The developing agents represented by the general formula are very useful as developing agents in the silver salt diffusion transfer process.

The negative materials employed in the invention may be film or paper having coated thereon black-white negative emulsions intended for use in usual photography or negative emulsions for use in X-ray photography. These negative emulsions contain silver halide, such as silver iodobromide, which may be spectrally and/or chemically sensitized. In addition, the positive materials are composed of a film or paper having coated thereon a layer containing nuclei of physical development. Among such positive materials is, for example, a "Positive Paper for Neo-Copy" made by Fuji Photo Film Co., Ltd.

The use of the compounds of the general formula in the processing solution for the high speed diffusion transfer process will be further illustrated by the following typical examples.

EXAMPLE 1

Between the silver halide emulsion layer, which was supported on a support and exposed to little exposure of exposure index ASA 1,000 and the print-receiving layer comprising a support having coated thereon silver-precipitant layer containing nuclei of physical development, was homogeneously spread a processing solution having the following, in thickness of about 30μ, and the diffusion transfer processings were conducted.

|                                               |     |       |
|-----------------------------------------------|-----|-------|
| H <sub>2</sub> O                              | ml. | 500.0 |
| Carboxymethyl cellulose (high viscosity)      | g.  | 20.0  |
| Na <sub>2</sub> SO <sub>3</sub>               | g.  | 30.0  |
| Na <sub>2</sub> S <sub>2</sub> O <sub>3</sub> | g.  | 20.0  |
| NaOH                                          | g.  | 20.0  |
| N,N-diethylhydroxylamine                      | ml. | 25.0  |
| Compound (1) (as hydrochloride)               | g.  | 15.0  |

After contact for about 30 seconds, the print-receiving layer was stripped to obtain a positive image of satisfactory gradation.

EXAMPLE 2

Example 1 was repeated, except that the following processing solution was used in place of the processing solution:

|                                               |     |       |
|-----------------------------------------------|-----|-------|
| H <sub>2</sub> O                              | ml. | 500.0 |
| Carboxymethyl cellulose (of high viscosity)   | g.  | 20.0  |
| Na <sub>2</sub> SO <sub>3</sub>               | g.  | 30.0  |
| Na <sub>2</sub> S <sub>2</sub> O <sub>3</sub> | g.  | 20.0  |
| NaOH                                          | g.  | 20.0  |
| N,N-diethylhydroxylamine                      | ml. | 25.0  |
| Compound (1) (as hydrochloride)               | g.  | 10.0  |

EXAMPLE 3

Example 1 was repeated, except that the processing solution was replaced by the following processing solution:

|                                               |     |       |
|-----------------------------------------------|-----|-------|
| H <sub>2</sub> O                              | ml. | 500.0 |
| Carboxymethyl cellulose (of high viscosity)   | g.  | 20.0  |
| Na <sub>2</sub> SO <sub>3</sub>               | g.  | 30.0  |
| Na <sub>2</sub> S <sub>2</sub> O <sub>3</sub> | g.  | 20.0  |
| NaOH                                          | g.  | 20.0  |
| p-Cresol                                      | ml. | 25.0  |
| Compound (1) (as hydrochloride)               | g.  | 10.0  |

EXAMPLE 4

Example 1 was repeated, except that compound (4) was employed as the hydrochloride in place of compound (1).

EXAMPLE 5

Example 2 was repeated, except that compound (4) was employed as the hydrochloride in place of compound (1).

EXAMPLE 6

Example 3 was repeated, except that compound (4) was employed as the hydrochloride in place of compound (1).

This invention has been described in detail with particular reference to preferred embodiments thereof but it will be understood that various variations and modifications can be effected within the spirit and scope of the invention as described and as defined in the appended claims.

What is claimed is:

1. A high speed diffusion transfer process which comprises processing an exposed photographic silver halide material with a processing solution containing a compound represented by the following general formula or acid salt thereof:



wherein X is a lower alkenyl or a lower alkoxy group, R<sub>1</sub> is hydrogen, or a lower alkyl group, and R<sub>2</sub>, R<sub>3</sub> and R<sub>4</sub> each is hydrogen, a lower alkyl group, a lower alkenyl group or a lower alkoxy group, in which the term "lower" indicates that the total number of carbon atoms is not more than 4.

2. The process as claimed in claim 1 wherein the processing solution contains ingredients capable of reacting with an unexposed silver halide to form the soluble silver complexes.

3. The process as claimed in claim 1 wherein the processing solution contains an alkaline agent, an antifoggant and/or viscosity-increasing agent thickeners.

4. The process as claimed in claim 1 wherein said compound or the acid addition salt thereof is employed singly in the processing solution.

5. The process as claimed in claim 1 wherein said compound or acid addition salt thereof is employed in combination with other reducing agents.

6. The process as claimed in claim 5 wherein said reducing agent is a hydroxylamine.

7. The process as claimed in claim 5 wherein the reducing agent is N,N-diethylhydroxylamine.

8. The process as claimed in claim 5 wherein said reducing agent is a phenol.

9. The process as claimed in claim 5 wherein the reducing agent is p-cresol.

10. The process as claimed in claim 1 wherein the compound is 4-amino-2-allylphenol, or salts thereof.

11. The process as claimed in claim 1 wherein the compound is 4-amino-2,6-diallylphenol, or salts thereof.

12. The process as claimed in claim 1 wherein the compound is 4 - amino - 2 - allyl-3,5-dimethylphenol, or salts thereof.

References Cited

UNITED STATES PATENTS

|    |           |         |               |       |         |
|----|-----------|---------|---------------|-------|---------|
| 5  | 3,186,843 | 6/1965  | Haas          | ----- | 96-66 R |
|    | 2,059,887 | 11/1936 | Manhes et al. | ----- | 96-59   |
|    | 2,652,428 | 9/1953  | Weissberger   | ----- | 96-66 X |
| 10 | 3,108,001 | 10/1963 | Green         | ----- | 96-66   |
|    | 3,241,964 | 3/1966  | Land          | ----- | 96-66 R |

NORMAN G. TORCHIN, Primary Examiner

U.S. Cl. X.R.

15 96-66 R